

No. 634,251.

Patented Oct. 3, 1899.

J. S. UNGER.

PROCESS OF CARBURIZING ARMOR PLATES.

(Application filed June 9, 1898.)

(No Model.)

2 Sheets—Sheet 1.



Fig. 1.

WITNESSES

Warren W. Swartz  
H. M. Corwin

INVENTOR

John S. Unger  
by Baxendell & Baxendell  
his Attorneys.

No. 634,251.

Patented Oct. 3, 1899.

J. S. UNGER.

PROCESS OF CARBURIZING ARMOR PLATES.

(Application filed June 9, 1898.)

(No Model.)

2 Sheets—Sheet 2.



WITNESSES

Warren U. Swartz,  
H. M. Corwin

INVENTOR

John S. Unger  
by Bannell & Bannell  
his Attorneys.

# UNITED STATES PATENT OFFICE.

JOHN S. UNGER, OF HOMESTEAD, PENNSYLVANIA, ASSIGNOR TO THE CARNEGIE STEEL COMPANY, LIMITED, OF PITTSBURG, PENNSYLVANIA.

## PROCESS OF CARBURIZING ARMOR-PLATES.

SPECIFICATION forming part of Letters Patent No. 634,251, dated October 3, 1899.

Application filed June 9, 1898. Serial No. 682,985. (No model.)

*To all whom it may concern:*

Be it known that I, JOHN S. UNGER, of Homestead, in the county of Allegheny and State of Pennsylvania, have invented a new and useful Improvement in Carburizing Armor-Plates, of which the following is a full, clear, and exact description, reference being had to the accompanying drawings, forming part of this specification, in which—

10 Figure 1 is a longitudinal sectional elevation of the gas-furnace or heating-chamber, showing the movable hearth in place. Fig. 2 is a horizontal section on the line II II of Fig. 1.

15 My invention relates to the supercarburization of plates or pieces of steel and is especially designed to be applied in the manufacture of armor-plate or of masses of steel to be shaped into armor-plate.

20 My invention is based on the discovery that carburization can be conducted most rapidly and most efficiently by using as the carburizing agent soot, the amorphous form in which carbon is deposited as the result of the de-  
25 composition of hydrocarbon gases.

I shall now describe the preferable mode of practicing my invention, referring to Fig. 1, in which 2 represents a heating-furnace having at the opposite sides gas-ports 3, through 30 which the heating-gas is introduced at one side of the furnace and discharged after combustion at the other side. 4 is a movable hearth common in furnaces of this type, carried on a truck 5, mounted on wheels 6 and 35 adapted to be moved into and out of the heating-chamber by a suitable motor 7. The plates of armor-steel are placed on the hearth with the faces to be carburized toward each other and separated by interposed billets or 40 supports 9. A gas-pipe 10, adapted to deliver hydrocarbon gas, is inserted into the space 11 between the armor-plates. An outlet for the gas is also provided at 12 by drilling at any convenient spot a hole, and said 45 space is sealed through one of its billets, and said space is otherwise sealed to exclude the air by luting with clay the joints between the billets. Intermediate sag-blocks, like the blocks 16, (shown in Fig. 2,) may also be em-  
50 ployed where the plates are of large area. This is the arrangement which has commonly

been adopted for supercarburizing armor-plate by the gas-treatment process. In such process it has been the practice first to heat the plates by the passage of flame through 55 the heating-chamber 2 until they are brought to a high temperature of about from 875° to 1,000° centigrade, and after the plates have been thus heated to introduce through the pipe 10 into the space between the plates a 60 current of hydrocarbon gas, which is caused to flow through the space and out of the outlet 12 for a period of six days or more, thus gradually carburizing the inner faces of the plates. When the gas thus introduced comes 65 into the highly-heated space between the plates, it is decomposed and deposits solid carbon upon the surfaces, and it is this deposited carbon which is absorbed by the metal and performs the work of carburization; but 70 the carbon thus deposited at the high temperature of the furnace is graphitic, and I have discovered that by modifying the conditions so that an initial layer of amorphous carbon or soot is deposited upon the faces of the steel 75 plates the carburizing operation can be conducted more rapidly and with better results than is otherwise possible. This I effect by introducing the hydrocarbon gas at an earlier stage than heretofore, while the armor-plate is 80 at a lower heat, such that the carbon will be deposited from the gas as amorphous carbon and not as graphite. Thus when the plate has been heated sufficiently to show a faint color, say a temperature of about 550° centigrade, I 85 introduce the hydrocarbon gas from the pipe 10. The consequence is that the faces of the plates will be covered with a layer of amorphous carbon or soot deposited from the gas, and when the plates afterward become more 90 highly heated and the carbon deposit becomes graphitic in its nature the graphitic carbon is deposited upon and as a covering for the inner layer of amorphous carbon. The layer of carbon next to the steel surface being 95 amorphous is in the most active and efficient condition in which it can be presented. The heating is continued and the temperature maintained at about 875° to 1,000° centigrade for six days or more, according to the thickness of the plates, until the desired degree of carburization has been effected. Specifically 100

I would state for the information of those practicing my invention that a plate six inches thick in a furnace constructed as shown in the drawings should be maintained at a temperature of 900° centigrade for about nine days or at 1,000° centigrade for about seven days in order to produce with my invention the degree of carburization ordinarily desired in armor-plate, the length of the operation necessary for different degrees of carburization being varied, as will be understood by those skilled in the art, accordingly as the temperature is kept at a higher or lower degree and as the plate treated is thicker or thinner. By my invention applied in this way the steel absorbs the carbon readily and quickly, enabling me to perform the work at lower temperature (say 900° centigrade) than has been common heretofore without unduly prolonging the operation and by using such lower temperature to avoid the danger of semifusing the surface of the plate, or when I use higher temperatures, say 900° to 1,000° centigrade, my invention enables me to perform the work in much less time than heretofore.

I believe I am the first to bring the gas into contact with the armor-plate to be carburized before the plates are brought to full working temperature of 875° to 1,000° centigrade.

I claim—

1. The process herein described for supercarburizing steel for armor-plates and other

purposes, which consists in heating the steel to a relatively low temperature, sufficient to cause the decomposition of hydrocarbon gas and the deposit therefrom of amorphous carbon or soot, bringing such gas into contact with the steel so heated, and excluding air, thereby depositing a layer of amorphous carbon upon the steel, then continuing at a higher temperature and for a period of days the heating of the plate and the admission of gas thereto, and depositing graphitic carbon upon the plate at such higher temperature; substantially as described.

2. The process herein described for supercarburizing steel for armor-plates and other purposes, which consists in introducing into contact with the steel hydrocarbon gas while the steel is at a temperature less than the working temperature of 875° to 1,000° centigrade, thereby causing a deposit of carbon at a relatively low heat, and then raising the temperature to the working point, continuing the heating and admission of gas for a period of days, and depositing graphitic carbon upon the plate at such higher temperature; substantially as described.

In testimony whereof I have hereunto set my hand.

JOHN S. UNGER.

Witnesses:

THOMAS W. BAKEWELL,  
H. M. CORWIN.